

April 1, 1941.

O. T. McILVAINE

2,236,647

ELECTRONIC TUBE

Original Filed Jan. 6, 1932

FIG.-1



FIG.-2



FIG.-3



INVENTOR  
O. T. MC ILVAINE  
BY *Harold Elmer Smith*  
ATTORNEY

## UNITED STATES PATENT OFFICE

2,236,647

## ELECTRONIC TUBE

Oran T. McIlvaine, Geneva, Ill.

Application January 6, 1932, Serial No. 584,967  
Renewed December 15, 1937

8 Claims. (Cl. 250—165)

This invention relates to electronic tubes and has among its objects the provision of a device of this character wherein an increased vigor of electronic emission is secured per unit of energizing intensity, either heat or light as the case may be; the provision of a photo-electron tube having greatly increased sensitiveness and volume of current; the provision of an energized electronic tube which shall be completely asymmetric in its action; the provision of an improved method of sensitizing or energizing such a tube; the provision of a new and improved composition of matter for effecting sensitization of such a tube; while further objects and advantages of the invention will become apparent as the description proceeds.

In the drawing accompanying and forming a part of this application Fig. 1 is a perspective view partly in section of an unfinished tube of preferred form containing my improvements although it will be understood that the tube in question is capable of very great modifications in the shape, size, arrangement, number, position, and relation of its active elements; Fig. 2 is a side elevation of a modified type of tube containing my improvements; and Fig. 3 is a section through a capsule of convenient shape together with its mounting.

In the particular embodiment here shown a cathode 1 and anode 2 are carried by a press 3 sealed in the stem 4 of a glass globe 5 and provided with leading-in wires 6. Any suitable or desirable kind of base can be employed.

In the embodiment shown in Fig. 1 the photo-electrode or cathode 1 consists of a metal plate 35 of substantially semi-cylindrical shape having the anode 2 substantially coinciding with its axis. This plate is carried by an upright post 7, the two electrodes being connected at their upper ends by a glass bridge 8 by which they are steadied, one of the parts also carrying a tiny hollow metallic capsule 9 in which the energizing substance or material is introduced. The cathode is preferably made, at least superficially, of silver and this preferably in a mat form. It may be a plate of pure silver, or it may equally well be a plate of base metal such as copper or nickel (or nickel-plated copper) electro-plated externally with silver. One well known method of accomplishing the production of a mat surface on an electro-plated article is by using a plating bath of silver cyanide. During the plating operation the current density is adjusted to the point where the desired character of surface is obtained on the plated article. Low current den-

sities tend to produce smoothly plated surfaces while high current densities tend to produce rough or mat surfaces, as is well understood by those skilled in the art. The anode can be of the same substance or any other conductive material, copper or nickel being especially desirable.

The energizing substance consists of a caesium compound mixed with one or more elemental substances of a type which react therewith at a red or white heat, but not at a lower temperature, to reduce the caesium compound to metallic caesium with the generation of reaction-products which are wholly solid. The employment of caesium as an energizing agent is not uncommon, nor is the employment of caesium produced by reaction, but a common procedure in the past has been to employ a reaction between caesium chloride and metallic calcium, thus producing calcium chloride and metallic caesium. Such mixture and reaction is unsatisfactory for two reasons: first, because caesium chloride tends readily to absorb water vapor which it is difficult or impossible to remove completely, and because the reaction between the calcium and the caesium chloride occurs at such low temperature as to render it impossible to heat the tube and its elements to a sufficient temperature to remove the occluded water vapor and other gases.

Accordingly an important feature of my invention is the employment of such an elemental substance in combination with such a compound of caesium that the reaction shall only occur at a temperature above that necessary for the successful outgassing of the tubes and the metallic elements and the energizing substance itself and this with the production of reaction products which are wholly solid, the ingredients also being of a non-hygroscopic nature. These considerations clearly eliminate all the gaseous, liquid, and easily fusible elements, all alkali- and alkaline-earth metals, all carbon, hydrogen, and halogen compounds, and leave in effect only oxygen-caesium compounds for the subject, and the higher-melting-point, oxygen-avid metals and metalloids as the reactive agents. The last-named limitation essentially eliminates such metals as copper, gold, platinum, silver and the iron-group metals, none of which have a strong affinity for oxygen. Aluminum lies nearly on the border line, being unsatisfactory in that its reaction tends to begin at too low a temperature and to proceed with undue vigor, although it can be employed in some cases if sufficiently diluted by restraining agents. Substances like boron, molybdenum,

tantalum and titanium are much better, but I prefer silicon above all; and for the caesium compound I prefer the chromate, inasmuch as it has a sufficiently high melting point, does not decompose or sublime while heating, is not hygroscopic, and produces, upon reaction with the substances mentioned, only solid non-volatile oxides. I do not limit myself to this one compound of caesium since other oxygen compounds thereof can be employed, such as the phosphate.

The preferred procedure is as follows: the caesium compound chosen, together with the reaction agent are mixed intimately together, preferably in the proper molecular proportions, and introduced into the capsule 9, which is made with a cavity for the purpose, the edges being closed by folding or spot-welding so as to hold the unreacted materials while allowing escape of volatilized caesium. The various elements are introduced and sealed into the glass globe, the air exhausted by way of the pipe 10 provided for the purpose, heat is applied in any suitable way to drive off the absorbed gases from the glass and from the tube elements, and a small amount of dry air (oxygen) is admitted, after which a uni-directional, high-tension current is passed between the anode and the cathode, from an induction coil or other uni-directional source whereby all combined oxygen is removed from the anode, and the surface of the cathode is covered with oxidized silver. The gases are then exhausted with the employment of sufficient heat to outgas the glass and metal and energizing substance without however producing the reaction of such substance.

Sufficient heat is then concentrated upon the capsule to produce a reaction between the substances therein, which in the preferred case consist of caesium chromate and silicon, the reaction products consisting of metallic caesium on the one hand and oxides of chromium and silicon on the other hand. The heating may be effected by a burning glass or by a high-frequency induction-furnace, and requires a bright red heat. It occurs without undue vigor, although a slight intensification of redness is visible at the instant of reaction. A distinct advantage of the described composition in the case of a photo electron tube is that the glass walls are left unobscured. The tube and its contents are now allowed to cool.

The leading-in wires are next connected to a suitable biasing battery in circuit with a microammeter and heat is applied to the tube by surrounding it with an internally heated jacket or other suitable means. As a result of the chemical reaction above described the metallic caesium will have become disseminated widely throughout the tube and upon cooling will have condensed on all parts of the same. The purpose of the heating is two-fold: first, to volatilize the caesium which has become deposited elsewhere than upon the cathode, by which alone it is absorbed and retained, due to the oxidation of the silver which is supposed to react in some way with the caesium; a second object of the heating is to produce the described reaction between the metallic caesium and the silver oxide. This reaction apparently varies with the temperature and is signalized by a continuous change in color of the cathode, and by a constant vibration of the ammeter needle as the temperature of the tube is gradually raised. The heating is stopped at the point at which the cathode exhibits the maximum photo-electric effect; this corresponds

to a yellowish color, often streaked or discolored with brown. Carried further than this the next color produced is a brown, also giving good photo-electric effects. If carried beyond this 5 the photo-electric effect will be found to decrease. The best mode of determining the proper point at which to stop is by allowing a beam of light of constant intensity to fall upon this photo-electrode alternatively with successive 10 heating periods, and arrest the heating as soon as the photo-electric current, as shown by the ammeter, begins to fall off.

I preferably employ lime-glass instead of lead-glass as the former permits the passage of more 15 of the ultra violet rays than does the latter, and I use either a vacuum or a gas-filling. Argon is good when gas is to be used, the pressures employed being up to a few mm. of mercury; 2/10 mm. pressure is very satisfactory, but either 20 more or less can be used.

As an example of a different arrangement I have shown in Fig. 2 a three-element tube comprising a photo-electrode 11, an anode 12, and a thermionic-electrode 13 (here consisting of an emissive element), the photo-electrode 11 also constituting a grid. The same procedure hereinabove described may be employed for energizing this tube, the grid 11 being first plated with silver before assembling, and oxidized during the pumping operation. This oxidation is confined 25 entirely to the photo-electrode or grid by the electrical protection of the other elements. The remaining steps are similar to those hereinbefore described. Such a tube, when subjected to a light-beam, will control passage of electrons from the thermionic-electrode 13 to the anode 12 in accordance with the intensity of the light-beam. A similar mode of operation could of course be obtained by connecting a separate thermionic- 30 electrode plate to this grid either in the same or a different tube. I mention these modifications here to show the flexibility of my process, and how any element out of many in a tube can be exclusively energized. It will be understood that 35 the energizing substance can be diluted with other substances, either active or inactive, beneficial or the reverse, without departing from my invention; for example a quantity of metallic chromium can be mixed with the other ingredients. Also the plating can be applied to the 40 cathode only or to both electrodes, since it is the oxidizing of the cathode surface and not its metallic nature which determines the selective adhesion of the caesium thereto. Other surfaces 45 than silver are operative for the purpose, though silver due to the ease with which it is electroplated and the weakness of its affinity for oxygen is particularly convenient. Accordingly I do not limit myself to the forms of elements 50 herein shown, nor the mode of connection thereof, nor the particular steps or materials described, except as the same are recited in my several claims which I desire may be construed broadly, each independent of limitations contained in other claims.

Having thus described my invention what I claim is:

1. A photo-electric tube comprising an anode and a silver-covered photo-electrode having a non-specular surface activated by caesium, the surface of said electrode exhibiting a color which lies between a straw color and a brown color.

2. A photo-electric tube comprising an anode and a silver-covered photo-electrode having a rough surface activated by caesium, the surface

of said electrode exhibiting in part a straw color and having patches of brownish color.

3. The art of manufacturing a photo-electric cathode comprising the steps of depositing a coating of oxidizable material on the surface of a foundation structure and so controlling the deposit as to produce a mat surface on the coating, oxidizing said mat surface, depositing on the oxidized surface a layer of light sensitive material, heating the cathode, and stopping the heating when the surface shows a desired color effect approximately between yellow and brown.

4. The process of activating an electrode of a photo-electric tube comprising the steps of electro-plating a coating of oxidizable material on the surface of a foundation structure and so controlling the electro-plating as to produce a mat surface on the coating, introducing said electrode into an envelope, oxidizing the mat surface of said electrode, depositing on the oxidized surface a layer of light sensitive material, producing a chemical reaction between the oxidized surface and the light sensitive material by heating the electrode, and stopping the heating when the surface shows a desired color effect approximately between yellow and brown.

5. The process of activating a cathode of a photo-electric tube comprising the steps of electro-plating a coating of oxidizable material on the surface of a foundation structure and so controlling the electro-plating as to produce a mat surface on the coating, introducing said cathode and caesium reaction mixture into an envelope, exhausting said envelope, oxidizing the surface of said cathode in the presence of oxygen, liberating the caesium from said caesium-reaction mixture and depositing the same on the cathode, heating the cathode, and stopping the heating

when the cathode shows a desired color effect approximately between yellow and brown.

6. The process of activating a cathode of a photo-electric tube comprising the steps of coating a foundation member with silver, producing a mat silver surface on said coating by electro-plating, introducing said cathode and a caesium reaction mixture into an envelope, exhausting said envelope, oxidizing the surface of the cathode in the presence of oxygen, liberating the caesium from said caesium reaction mixture and depositing the same on the cathode, heating the cathode with the caesium deposit thereon, and stopping the heating when the cathode shows a color approximately between yellow and brown.

7. The art of manufacturing a photo-electric cathode comprising the steps of depositing a coating of oxidizable material on the surface of a foundation structure and so controlling the deposit as to produce a mat surface on the coating, oxidizing said mat surface, depositing on the oxidized surface a layer of light sensitive material, producing a chemical reaction between the oxidized surface and the light sensitive material by applying heat to the cathode, and stopping the heating when the surface shows a color effect approximately between yellow and brown.

8. The process of manufacturing a photo-electric cathode comprising the steps of depositing a coating of oxidizable material on the surface of a foundation structure and so controlling the deposit as to produce a mat surface on the coating, oxidizing said mat surface, depositing on the oxidized surface a layer of light sensitive material, heating the cathode, and stopping the heating when the surface shows a desired color effect.

ORAN T. McILVAINE.